

## UNITED STATES PATENT OFFICE

2,204,535

## FIBER

Stephen P. Gould and Earle O. Whittier, Washington, D. C.; dedicated to the free use of the People in the territory of the United States

No Drawing. Application May 28, 1938,  
Serial No. 210,790

## 1 Claim. (Cl. 28—1)

(Granted under the act of March 3, 1883, as amended April 30, 1928; 370 O. G. 757)

This application is made under the act of March 3, 1883, as amended by the act of April 30, 1928, and the invention herein described and claimed, if patented, may be manufactured and used by or for the Government of the United States of America for governmental purposes without the payment to us of any royalty thereon.

We hereby dedicate the invention herein described to the free use of the People in the territory of the United States to take effect on the granting of a patent to us.

Our invention pertains to fibers composed essentially of casein and containing a relatively high percentage of metallic salts.

The object of our invention is to produce compositions, suitable for spinning into fibers, comprising casein and metallic caseinates in soluble form, and containing a high percentage of metallic compounds. Thus the strength, water-resistance, and elasticity of said fibers are greatly increased. Other objects will become apparent in the course of the following teachings.

In forming dispersions containing casein, suitable for spinning into fibers, it is difficult to incorporate more than a comparatively small amount, as about 3% (based on the weight of the casein), for instance, of strengthening and water-resisting salts, such as calcium chloride, without causing precipitation of calcium caseinate. This prevents the spinning of the dispersion. If, however, sulfated or sulfonated (preferably to a considerable degree) aliphatic or aromatic compounds, as for example, a sulfated vegetable oil, are incorporated with the dispersion much larger amounts of metallic compounds may be blended into the composition without the precipitation of the corresponding caseinate. If sodium hexametaphosphate, pyrophosphate, or a mixture of these is added to the casein composition, even larger amounts (20-30%) of the metallic compounds may be mixed with the dispersion without the separation of insoluble metallic caseinates.

Inorganic bisulfites, such as those of sodium and ammonium, are often useful in obtaining smooth casein dispersions of high metallic content. In the presence of these bisulfites, non-sulfated oils, such as oleic acid, are often compatible with the spinning solution.

If the metallic compound used is calcium hydroxide, careful filtration is required to avoid plugging the spinnerette holes. Comparatively large amounts of amphoteric compounds, such as sodium aluminate, may be incorporated without a too great increase in viscosity if the spinning dispersion comprises the previously men-

tioned high-percentage sulfur trioxide-containing compounds and/or phosphates. Without these compounds, the addition of sodium aluminate, for instance, in increasing amounts above 2%, results in a rapidly increasing viscosity of the solution so that it cannot be easily spun. Barium hydroxide is one of the most satisfactory of the metallic compounds to use because of its greater solubility and because the fiber retains a high proportion of its barium while in the precipitating bath.

The following examples are given to illustrate some preferred methods for insuring the compatibility of large amounts of metallic caseinates with spinning solutions. Proportions are given in parts.

## EXAMPLE I

## Spinning solution

|                                                                       |        |    |
|-----------------------------------------------------------------------|--------|----|
| Casein                                                                | 24     | 20 |
| Water                                                                 | 100    | 20 |
| A highly sulfonated vegetable oil (or its sodium salt)                | 3.6    |    |
| A mixture of sodium hexametaphosphate and pyrophosphate               | 1.5    |    |
| Barium hydroxide $[\text{Ba}(\text{OH})_2 \cdot 8\text{H}_2\text{O}]$ | 4.42   | 25 |
| Water                                                                 | 106.48 |    |

The 24 parts of casein are soaked in the 100 pts. of water for 15-30 minutes. The sulfated oil and the phosphates are then added and the mixture warmed until the casein is largely dissolved. The barium hydroxide is then dissolved in the remaining quantity of water, and the solution stirred mechanically into the casein composition. Thus a smooth dispersion is obtained, free from lumps of insoluble caseinate.

The temperature of both the spinning solution and the precipitating bath was 50° C. However, other temperatures varying from room to 80° C. may be used.

The sulfated oil serves also as a plasticizer. If even softer fibers are desired, the amount of the oil may be increased, or the fibers may be subjected to an after treatment with oil, glycerol, or similar softening material.

The bath composition is:

|               | Parts |
|---------------|-------|
| Sulfuric acid | 8     |
| Formaldehyde  | 5     |
| Dextrose      | 20    |
| Water         | 67    |

This bath composition may, however, be varied.

The above procedure for incorporating large amounts of metallic compounds into the spinning

solution results in fibers of greater strength and water resistance.

The following example illustrates the use of a sulfonated aromatic product, and of a high percentage of a calcium salt.

EXAMPLE 2

|                                   |       |
|-----------------------------------|-------|
| Casein                            | 24    |
| Water                             | 160.5 |
| 10 Sodium hydroxide solution (2N) | 8     |
| Calcium cymene sulfonate          | 7.5   |

Additional plasticizers may be added if a softer product is desired or the fibers may be after treated with oils.

15 Example 3 illustrates the use of a high percentage of sodium aluminate. Such solutions are ordinarily too viscous to spin, but in this case, the sulfated oil and hexametaphosphate present enable this to be done.

EXAMPLE 3

|                                                         |      |
|---------------------------------------------------------|------|
| Casein                                                  | 24   |
| Water                                                   | 125  |
| Sodium hydroxide solution (2N)                          | 8    |
| 25 A highly sulfated vegetable oil (or its sodium salt) | 4.8  |
| Sodium hexametaphosphate                                | 1.5  |
| Sodium aluminate                                        | 3.6  |
| Water                                                   | 99.1 |

30 Casein may be sulfonated directly by the action of chlorosulfonic acid whereby the insolubility of the metallic caseinates may be increased. The chlorosulfonic acid is stirred directly into the dry casein; allowed to react for a short time, 15 minutes, for example, and water is then cautiously added. The alkali should be added promptly to minimize the effect of the hydrochloric acid liberated by the reaction.

EXAMPLE 4

|                                                           |       |
|-----------------------------------------------------------|-------|
| Casein                                                    | 24    |
| Chlorosulfonic acid                                       | 2.0   |
| Water                                                     | 100   |
| Oleic acid                                                | 3.6   |
| Sodium hexametaphosphate                                  | 1.5   |
| 45 Sodium hydroxide solution (2N)                         | 15    |
| Barium hydroxide [Ba(OH) <sub>2</sub> ·8H <sub>2</sub> O] | 4.42  |
| Water                                                     | 89.48 |

If the amount of chlorosulfonic acid is increased, the sodium hexametaphosphate may be omitted.

Example 5 illustrates the use of a sulfated higher alcohol in increasing the compatibility of the metallic compounds with the casein composition.

EXAMPLE 5

|                                                           |        |
|-----------------------------------------------------------|--------|
| Casein                                                    | 24     |
| Water                                                     | 100    |
| Sodium oleyl sulfate                                      | 3.6    |
| Sodium hexameta- and pyrophosphate mixture                | 2.4    |
| Barium hydroxide [Ba(OH) <sub>2</sub> ·8H <sub>2</sub> O] | 6.64   |
| Water                                                     | 103.36 |

The bath composition and temperatures are the same for Examples 2-5, inclusive, as those given under Example 1.

The flexibility of these fibers may be improved by incorporation of an oil or fat with the sodium oleyl sulfate or by after treatment with oils or glycerin.

It will be understood that our invention is not limited to the above examples as proportions, constituents, and substitutes may be varied over a wide range. It is also possible at some concentrations to omit certain ingredients, such as, for instance, the mixture of phosphates. The amounts of metallic compounds may particularly be varied, and similar amphoteric compounds may be substituted for the sodium aluminate.

The general procedure is the same in the case of all the examples, i. e., the spinning solutions are extruded through any type of spinnerette normally used in the rayon industry into precipitating baths of the indicated compositions.

Having thus described our invention, what we claim for Letters Patent is:

As an article of manufacture, a fiber comprising casein, sulfonated casein, salts of sulfonated casein and of casein as its essential components; and fat acids.

STEPHEN P. GOULD.  
EARLE O. WHITTIER.